

# UNITED STATES PATENT OFFICE.

HUGH RODMAN, OF EDGEWOOD, PENNSYLVANIA, ASSIGNOR TO RODMAN CHEMICAL COMPANY, OF VERONA, PENNSYLVANIA, A CORPORATION OF PENNSYLVANIA.

## CARBURIZING MATERIAL.

1,279,160.

Specification of Letters Patent. Patented Sept. 17, 1918.

No Drawing.

Application filed July 9, 1914. Serial No. 850,067.

*To all whom it may concern:*

Be it known that I, HUGH RODMAN, a citizen of the United States, and a resident of Edgewood, in the county of Allegheny and State of Pennsylvania, have made a new and useful Invention in Carburizing Material, of which the following is a specification.

This invention has to do with the art of carburizing steel by dry packing, and discloses a new and useful material therefor and a method of manufacturing this material.

The essence of the invention lies in the observation that only the surface of granular carburizing material is highly active and in the conception that improved material may therefore be constructed by coating an inert, or comparatively inert, particle or small mass with a highly active covering material.

By this means many advantages are secured. The centers may be selected for strength, cheapness, thermal conductivity, permanency of volume, etc., without reference to carburizing efficiency, and materials which are ordinarily impracticable because of mechanical weakness or cost may be utilized as coating material, the inert, or comparatively inert centers furnishing the necessary mechanical strength and the reduced amount of active material lowering the total cost.

It is desirable, though not essential, that the covering material should contain no substance that will fuse and flow into the body of the centers, as the carburizing strength of the coating would thereby be reduced. I therefore prefer to avoid the use of fusible material, such as the various sodium or potassium compounds ordinarily used in carburizing mixtures, and to rather use such infusible compounds as barium carbonate and calcium hydroxid, these being mixed with appropriate amounts of carbonaceous materials such as powdered coal or powdered leather char. For the inert centers I prefer ordinary metallurgical coke, as it is cheap, light, permanent, conductive, etc., but other materials, such as crushed brick, charcoal, etc., may be used if desired.

As a concrete and successful example of my invention I will cite the following, but

with no idea of limiting the invention to the specific materials or proportions enumerated.

I tumble 1000 pounds of coke particles, screened between  $\frac{1}{4}$ " and  $\frac{1}{8}$ " openings, with about 100 pounds of molasses solution approximately 1.1 density. I then gradually add about 400 pounds of coating mixture consisting of 100 parts powdered coal, 100 parts Portland cement, 10 parts calcium hydroxid and 25 parts barium carbonate and continue the tumbling till the coke centers are all well covered and smooth. I then spread the material on the floor to dry and harden for about twenty-four hours.

It will be apparent that some reaction between the coke or carbonaceous centers and the chemical energizers may take place and some small carburizing effect may therefore be produced, but the carbonaceous coating produces practically all of the carburizing effect. In fact where such centers have intrinsically some slight carburizing qualities (when used alone) as in the case of charcoal, I believe the coating applied not only produces substantially all the carburizing effect, but actually cloaks or lessens the carburizing effect intrinsically possessed by the centers. Where a fusible energizer is used and where therefore some of the energizer flows into the carbonaceous center, the carburizing properties of the center are still negligible because they are cloaked by the applied coating of a highly active material.

Other materials and proportions will occur to those skilled in the art. For instance, the binder may be tar or other hydrocarbons, the covering may be powdered leather char or bone black: the essential idea being that the activity of the material shall principally reside in the coating applied to the inert, or comparatively inert, centers.

Having thus described my invention, what I claim is:

1. A carburizing material consisting of small masses, and a material in itself highly active as a carburizing agent forming a coating for each of said masses.

2. A carburizing material consisting of carbonaceous masses, and a material in itself highly active as a carburizing agent forming an active carburizing coating for each of said masses.

3. A carburizing material consisting of carbonaceous masses having little or no carburizing properties, and a material highly active as a carburizing material forming a 5 coating for each of said masses and cloaking the carburizing activity of the masses.
4. A carburizing material consisting of a relatively inert carbonaceous mass having bound thereto a permanent coating of energized carbon material.
5. A carburizing material consisting of small masses, coated with a coating of powdered carbonaceous material and an energizing material.
- 15 6. A carburizing material consisting of small masses having little or no carburizing properties, and an active coating for each of said masses comprising powdered carbonaceous material, an energizer, and a binder.
- 20 7. A carburizing material consisting of small inert masses and an active coating of carburizing material for each of said masses.
8. A carburizing material consisting of small coke masses and a permanent active coating for each of said masses containing 25 carbonaceous material and an infusible energizer.
9. A carburizing material consisting of small masses having little or no carburizing properties, and an active coating for said 30 masses comprising powdered animal char, an energizer and a binder.

In testimony whereof, I have hereunto subscribed my name this 7th day of July, 1914.

HUGH RODMAN.

Witnesses:

E. W. McCALLISTER,  
ANNA CLOHERTY.